

## UNITED STATES PATENT OFFICE.

JULIAN L. SCHUELER, OF PEORIA, ILLINOIS.

## PROCESS OF MAKING BASIC OPEN-HEARTH STEEL.

No Drawing.

Application filed March 27, 1926. Serial No. 98,018.

- This invention has reference to a process for making basic open hearth steel and has special reference to the making of steel starting with a cold metallic charge.
- 5 My improved process consists in so charging a heat that the amount of limestone charged is materially reduced and the charge will melt in less time than is usual with charges of this character.
- 10 A further object of my process consists in reducing the amount of coke, pig iron, cast iron or other carbon giving materials usually needed in charges of this character.
- 15 A further object of my process is that the melting of the heat (high in carbon or low in carbon) may be controlled within rather narrow limits.
- 20 A further object of my process is the reduction in the amount of fuel necessary to melt the charge.
- The foregoing objects are attained by charging the heats as is usual for charges of this character, except that only about half or less of the amount of limestone usually 25 charged is added. On account of the lessened amount of stone charged a considerably less amount of carbon is needed in the bath to bring the stone up, as will be well understood by those skilled in the art. I
- 30 may, of course, charge burned lime instead of limestone, in which case the amount of carbon is reduced over that necessary with limestone, and it is possible for the heats to be made in lessened time. The amounts 35 to be used will be readily apparent to those skilled in the art from the description of the practice as outlined with limestone given below.
- Then, on account of this lessened stone, it 40 is obvious that as soon as the charge melts the limestone will all be up in the slag. Thus a considerable saving of fuel results from the lessened melting time.
- With this lessened amount of limestone 45 the slag formed is very thin, so as soon as the heat has melted I add burned lime which quickly brings the slag up to the proper consistency. Then after adding any other furnace additions, such, for example, as spiegel or ferro-manganese, the heat is ready to tap.
- For example, in the usual practice limestone is charged, equal to from 9 to 14 per cent of the weight of the metal charged. In 50 my improved process I charge only 3½ to 7 per cent of the weight of the charge, as limestone. Furthermore, if coke is used to fur-
- nish a part of the carbon by use of my process I cut this from 3.5 per cent of the weight of the charge to 2.5 per cent, a very material reduction. Or if pig iron or cast iron, 60 or both, are used I may cut these down proportionately (depending on their carbon content) instead of the coke, or I may cut down on all three in the proportion outlined above. Furthermore, heats of this type, 65 which are usually made in 13 to 14 hours, are made by my process in from 11 to 12½ hours. With a furnace using oil as a fuel I am able by my process to cut the consumption of oil from about 56 gallons per ton to about 50 70 gallons per ton. When using burned lime I charge from 1½ to 5 per cent of the weight of the metal charged. It is obvious, therefore, that I can use either limestone or burned lime and it is, also, obvious to those 75 skilled in the art that when substituting burned lime for limestone I would use less carbon giving materials.
- I have found by actual practice over an extended period of time that the process as 80 described above, and the objects as outlined, are attained in a very efficient manner, and the cost of making steel by my process is materially less than that made by the usual and ordinary process.
- 85 What I claim is:—
1. The process of making basic open hearth steel using cold charges, which consists in first charging an insufficient amount of limestone to form a finishing slag with 90 respect to the weight and kind of metal charged, and without removing the slag formed, finally making up the insufficiency of limestone after the charge has melted by the addition of burned lime to form the 95 finishing slag.
  2. The process of making basic open hearth steel using cold charges, which consists in first charging an insufficient amount of limestone to form a finishing slag, the 100 weight of the limestone being equivalent to between 3½ and 7 per cent with respect to the weight and kind of metal charged, and without removing the slag formed, finally making up the insufficiency of limestone, 105 after the charge has melted by the addition of burned lime to form the finishing slag.
  3. The process of making basic open hearth steel using cold charges, which consists in first charging an insufficient amount of limestone to form a finishing slag with 110 respect to the weight and kind of metal

charged, adding a suitable lessened amount of carbon-giving materials to conform to the lessened amount of limestone, and without removing the slag formed, finally making up the insufficiency of limestone after the charge has melted by the addition of burned lime to form the finishing slag.

4. The process of making basic open hearth steel using cold charges, which consists in first charging an insufficient amount of limestone to form a finishing slag, the weight of the limestone being equivalent to between 3½ and 7 per cent with respect to the weight and kind of metal charged, adding a suitable lessened amount of carbon-giving materials to conform to the lessened amount of limestone, and without removing the slag formed, finally making up the insufficiency of limestone after the charge has melted by the addition of burned lime to form the finishing slag.

5. The process of making basic open hearth steel using cold charges, which consists in first charging an insufficient amount of burned lime to form a finishing slag with respect to the weight and kind of metal charged, and without removing the slag formed, finally making up the insufficiency of burned lime after the charge has melted by a further addition of burned lime to form the finishing slag.

6. The process of making basic open hearth steel using cold charges, which consists in first charging an insufficient amount of burned lime to form a finishing slag, the weight of the burned lime being equivalent

to between 1½ and 5 per cent with respect to the weight and kind of metal charged, and without removing the slag formed, finally making up the insufficiency of burned lime after the charge has melted by a further addition of burned lime to form the finishing slag.

7. The process of making basic open hearth steel using cold charges, which consists in first charging an insufficient amount of burned lime to form a finishing slag with respect to the weight and kind of metal charged, adding a suitable lessened amount of carbon-giving materials to conform to the lessened amount of burned lime, and without removing the slag formed, finally making up the insufficiency of limestone after the charge has melted by a further addition of burned lime to form the finishing slag.

8. The process of making basic open hearth steel using cold charges, which consists in first charging an insufficient amount of burned lime to form a finishing slag, the weight of the burned lime being equivalent to between 1½ and 5 per cent with respect to the weight and kind of metal charged, adding a suitable lessened amount of carbon-giving materials to conform to the lessened amount of burned lime, and without removing the slag formed, finally making up the insufficiency of burned lime after the charge has melted by a further addition of burned lime to form the finishing slag.

JULIAN L. SCHUELER.